# EUROPEAN PATENT SPECIFICATION

(11) **EP 3 031 056 B1**
(45) Date of publication and mention of the grant of the patent: **13.09.2017**
(21) Application number: 14744112.5
(22) Date of filing: 28.07.2014
(51) Int. Cl.: H01F 1/01

(54) **MAGNETOCALORIC MATERIALS CONTAINING B**
MAGNETOKALORISCHES MATERIAL ENTHALTEND B
MATÉRIAU MAGNÉTOCALORIQUE CONTENANT B

(30) Priority: 09.08.2013 EP 13179965
(43) Date of publication of application: 15.06.2016
(73) Proprietor: BASF SE, 67056 Ludwigshafen am Rhein (DE)
(72) Inventor: GUILLOU, Francois, NL-2645 GA Delfgauw (NL); BRUECK, Ekkehard, NL-2628AH Delft (NL); REESINK, Bernard Hendrik, NL-7107 AD Winterswijk-Kotten (NL)
(86) International application number: PCT/EP2014/066132
(87) International publication number: WO 2015/018678

(56) References cited:
- CN-A- 102 881 393
- DATABASE INSPEC [Online] THE INSTITUTION OF ELECTRICAL ENGINEERS, STEVENAGE, GB; March 2011 (2011-03), WANG DONGMEI ET AL: "Magnetocaloric effect in MnFeP0.63Ge0.12Si0.25Bx (x=0, 0.01, 0.02, 0.03) compounds", XP002730497, Database accession no. 12840565 & ACTA METALLURGICA SINICA SCIENCE PRESS CHINA, vol. 47, no. 3, March 2011 (2011-03), pages 344-348, ISSN: 0412-1961, DOI: 10.3724/SP.J.1037.2010.00566
- FRANÇOIS GUILLOU ET AL: "Taming the First-Order Transition in Giant Magnetocaloric Materials", ADVANCED MATERIALS, vol. 26, no. 17, 22 May 2014 (2014-05-22), pages 2671-2675, XP055143389, ISSN: 0935-9648, DOI: 10.1002/adma.201304788
- GUILLOU F ET AL: "Magnetocaloric effect, cyclability and coefficient of refrigerant performance in the MnFe(P, Si, B) system", JOURNAL OF APPLIED PHYSICS, AMERICAN INSTITUTE OF PHYSICS, US, vol. 116, no. 6, 14 August 2014 (2014-08-14), XP012188611, ISSN: 0021-8979, DOI: 10.1063/1.4892406 [retrieved on 1901-01-01]
- F. GUILLOU ET AL: "About the mechanical stability of MnFe(P,Si,B) giant-magnetocaloric materials", JOURNAL OF ALLOYS AND COMPOUNDS, vol. 617, 1 September 2014 (2014-09-01), pages 569-574, XP055143384, ISSN: 0925-8388, DOI: 10.1016/j.jallcom.2014.08.061

## Description

The present invention relates to materials having a large magnetocaloric effect (MCE), more precisely to those materials combining a large entropy change, a large adiabatic temperature change, a limited hysteresis and excellent mechanical stability; and also to the processes for preparing/producing such materials.

In magnetic materials, magnetic phase transitions manifest themselves by an anomaly on the entropy versus temperature curve, that is to say by an entropy rise. Due to the intrinsic sensitivity of magnetic phase transitions to the application of an external magnetic field, it is possible to shift in temperature this entropy anomaly by a magnetic field change. Depending on whether the field change is performed in isothermal or adiabatic conditions, the effect is quantified either as an entropy change (ΔS) or an adiabatic temperature change (ΔT_{ad}) and is called magnetocaloric effect (MCE). For a ferromagnetic compound around the Curie temperature (T_{C}), increasing the magnetic field leads to a shift of the entropy anomaly toward higher temperatures, the resulting MCE is thus a negative entropy change and a positive temperature change. Magnetic phase transitions can be induced either by a magnetic field change or by a temperature change.

Systems using the magnetocaloric effect cover a broad range of practical applications, from thermomagnetic devices wherein the machine converts a thermal energy into a magnetic work, to heat pumps wherein magnetic work is used to transfer thermal energy from a cold source to a hot sink or vice versa. The former type includes devices that use in a second step the magnetic work: to produce electricity (generally referred to as thermomagnetic, thermoelectric and pyromagnetic generators) or to create a mechanical work (like thermo-magnetic motors). While the latter type corresponds to magnetic refrigerators, heat exchangers, heat pumps or air conditioning systems.

For all these devices it is of primary interest to optimize the heart of the device, the MCE material, also called magnetocaloric material. This MCE is quantified either as an entropy change (ΔS) or a temperature change (ΔT_{ad}), depending on whether the field application is performed in isothermal or in adiabatic conditions, respectively. Often only the ΔS is considered, but since there is no direct relation linking these two quantities, there is no reason to give a preference to only one parameter and thus, it is required to simultaneously optimize both.

All the MCE applications previously cited have a cyclic character, i.e. the magnetocaloric material runs through the magnetic phase transition frequently, it is thus important to ensure the reversibility of the MCE when either field or temperature oscillations are applied. This means that the magnetic field or thermal hysteresis which could take place around the MCE has to be kept low.

From a practical point of view, in order to allow large-scale applications, the MCE material must be formed of elements available in large amounts, not expensive and not classified as toxic.

For applications using the MCE caused by application of magnetic field changes, the MCE must be preferably achieved by magnetic field changes of the order of what can be provided by permanent magnet such as ΔB ≤ 2 T, and more preferably ΔB ≤ 1.4 T.

Another practical requirement for applications is related to the mechanical stability of the material. The fact is that the most attractive MCE materials take advantage from the discontinuous change in magnetization occurring at first order transitions. However, first order transitions lead to discontinuities on other physical parameters including the unit cell in case of solid materials having a crystalline structure. This "structural" part of the transition could give manifold changes: symmetry breaking, cell volume change or anisotropic cell parameters changes etc. The most dramatic parameter for the stability of bulk polycrystalline samples turns out to be the cell volume change. During thermal or magnetic field cycling, the strains generated by a volume change lead to fractures or a destruction of the bulk piece, which can severely hinder the applicability of these materials. Having a zero volume change at the first order transition is thus a first step to ensure a good mechanical stability.

US 7,069,729 presents magnetocaloric materials of the general formula MnFe(P₁₋ₓAsₓ), MnFe(P₁₋ₓSbₓ) and MnFeP_{0.45}As_{0.45}(Si/Ge)_{0.10} which, generally, do not fulfil the toxicity condition.

US 8,211,326 discloses magnetocaloric materials of general formula MnFe(P_{w}GeₓSi_{z}) which include a critical element (Ge, scarce and expensive) improper for large scale applications.

US 2011/0167837 and US 2011/0220838 disclose magnetocaloric materials of general formula (MnₓFe₁₋ₓ)_{2+z}P_{1-y}Si_{y}. These materials have a significant ΔS but not necessarily the combination of large ΔS and large ΔT_{ad} suitable for most of the applications. Materials having a manganese to iron ratio (Mn/Fe) of 1 show large hystereris. This is disadvantageous in respect to the application of the magnetocaloric effect in machines with cyclic operation. Changing the manganese to iron ratio (Mn/Fe) away from 1 leads to a decrease of the hysteresis. Unfortunately it turns out that the improvement in respect to hysteresis is paid by a decrease of the saturation magnetization, see N.H. Dung et al. Phys. Rev. B 86, 045134 (2012), which is undesired since for MCE purposes the magnetization of the magnetocaloric material should be as high as possible.

CN 102881393 A describes Mn_{1.2}Fe_{0.8}P_{1-y}Si_{y}B_{z} with 0.4 ≤ y ≤ 0.55 and 0 ≤ z ≤ 0.05. According to the data shown the addition of B seems to shift the Curie temperature of the materials towards higher temperatures, but seems to have no effect on the hysteresis according to the experimental data presented. ΔT_{ad} values achievable in magnetic cooling operations with the materials described are not disclosed.

It was the object of the present invention to provide magnetocaloric materials having a broad range of working temperatures (preferably from 150 K to 370 K) and combining large ΔS and ΔT_{ad} in intermediate fields (ΔB ≤ 2 T, preferably 4B ≤ 1.4 T), a limited hysteresis and a limited cell volume change.

This object is achieved, according to claim 1, by magnetocaloric materials of the general formula (I)

(MnₓFe₁₋ₓ)₂₊ᵤ P_{1-y-z}Si_{y}B_{z}

wherein
0.55 ≤ x ≤ 0.75,
0.25 ≤ y < 0.4,
0.05 < z ≤ 0.2,
-0.1 ≤ u ≤ 0.05.
A further aspect of the present invention relates to a process for producing such magnetocaloric materials, according to claim 10, the use of such magnetocaloric materials in cooling systems, heat exchangers, heat pumps or thermoelectric generators, according to claim 13, and cooling systems, heat exchangers, heat pumps or thermoelectric generators containing the inventive magnetocaloric materials, according to claims 14.
The inventive magnetocaloric materials are formed from elements which are generally classified as non-toxic and non-critical. The working temperature of the inventive magnetocaloric materials is in the range from -150 °C to +50 °C which is beneficial for use in a wide range of cooling applications like refrigerators and air conditioning. The inventive magnetocaloric materials have very beneficial magnetocaloric properties; in particular they exhibit large values of ΔS and at the same time large values of ΔT_{ad} and show very low thermal hysteresis. Furthermore, the inventive materials undergo only very small or practically no cell volume change during the magnetic phase transition. This leads to a higher mechanical stability of the materials during continuous cycling which is mandatory for actual application of magnetocaloric materials.
The stoichiometric value x is at least 0.55, preferably at least 0.6. The maximum value for x is 0.75, preferred 0.7. Especially preferred is the range 0.6 ≤ x ≤ 0.7.
The stoichiometric value y is at least 0.25, preferably at least 0.3, more preferred at least 0.32. The maximum value of y is 0.4, preferably the maximum value of y is 0.36, and more preferred the maximum value of y is 0.34. Preferred is the range 0.3 ≤ y < 0.4, more preferred is the range 0.3 ≤ y ≤ 0.36, and especially preferred is the range 0.32 ≤ y ≤ 0.34.
The lower limit of the stoichiometric value z is > 0.05, preferably z is at least 0.052 and more preferred z is at least 0.06. The maximum value of z is 0.2, preferably 0.16, more preferred 0.1 and particularly preferred the maximum value of z is 0.09. A preferred range of z is 0.052 ≤ z ≤ 0.1, more preferred 0.06 ≤ z ≤ 0.09.

The stoichiometric value u may differ from 0 by small values, u is usually -0.1 ≤ u ≤ 0.05, preferably -0.1 ≤ u ≤ 0, more preferred -0.05 ≤ u ≤ 0 and in particular -0.06 ≤ u ≤ -0.04.

One advantage of the present inventive materials is the possibility to easily get a limited hysteresis by balancing simultaneously Mn/Fe and P/Si ratios with a fine adjustment of z. In this respect, it should be noted that in the materials according to the present invention the substitution of Phosphorous by Boron has a large influence on the thermal hysteresis (c.f. examples), a result in stark contrast with the B addition shown in CN 102881393 A, where all the provided experimental examples display an undesired large thermal hysteresis. For cyclically operated devices, the thermal hysteresis should not exceed the adiabatic temperature change induced by the available magnetic field. The thermal hysteresis (in zero magnetic field) is preferably ≤ 6 °C, more preferably ≤ 3 °C.
Inventive materials showing especially good properties in respect to the simultaneous presence of large values of ΔS and ΔT_{ad}, small hysteresis and small cell volume change at T_{c} are magnetocaloric materials of formula (I) wherein
0.6 ≤ x ≤ 0.7,
0.3 ≤ y < 0.4, preferably 0.30 ≤ y ≤ 0.36, most preferred 0.32 ≤ y ≤ 0.34, and
0.052 ≤ z ≤ 0.1, preferably 0.06 ≤ z ≤ 0.09.

These magnetocaloric materials have a Si content close to 1/3 which is especially favourable to get Curie Temperature below room temperature (- 150 °C to 20°C). A second advantage of this range lays in the high magnetization values that are found when y≈ 1/3 [Z. Ou, J. Mag. Mag. Mat. 340, 80 (2013)]. In such a case, the best materials showing limited thermal hysteresis are obtained if z is at least 0.06, as found by the inventors and shown in the examples.

The inventive magnetocaloric materials have preferably the hexagonal crystalline structure of the Fe₂P type.

The inventive magnetocaloric materials exhibit only small or practical no volume change at the magnetic phase transition whereas similar boron free magnetocaloric materials clearly show volume steps at the magnetic phase transition. Preferably, the inventive magnetocaloric materials exhibit a relative volume change |ΔV/V| at the magnetic phase transition of at maximum 0.05 %, more preferred of at maximum 0.01 %, most preferred the maximum value of |ΔV/V| is equal to the value caused by the mere thermal expansion of the inventive magnetocaloric material at the magnetic phase transition. The value of |ΔV/V| may be determined by X-ray diffraction.

The inventive magnetocaloric materials may be prepared in any suitable manner. The inventive magnetocaloric materials may be produced by solid phase conversion or liquid phase conversion of the starting elements or starting alloys for the magnetocaloric material, subsequently cooling, optionally pressing, sintering and heat treating in one or several steps under inert gas atmosphere and subsequently cooling to room temperature, or by melt spinning of a melt of the starting elements or starting alloys.

Preferably the starting materials are selected from the elements Mn, Fe, P, B and Si, i.e. from Mn, Fe, P, B and Si in elemental form, and from the alloys and compounds formed by said elements among each other. Non-limiting examples of such compounds and alloys formed by the elements Mn, Fe, P, B and Si are Mn₂P, Fe₂P, Fe₂Si and Fe₂B.

Solid phase reaction of the starting elements or starting alloys may be performed in a ball mill. For example, suitable amounts of Mn, Fe, P, B and Si in elemental form or in the form of preliminary alloys such as Mn₂P, Fe₂P or Fe₂B are ground in a ball mill. Afterwards, the powders are pressed and sintered under a protective gas atmosphere at temperatures in the range from 900 to 1300° C, preferably at about 1100° C, for a suitable time, preferably 1 to 5 hours, especially about 2 hours. After sintering the materials are heat treated at temperatures in the range from 700 to 1000° C, preferably about 950° C, for suitable periods, for example 1 to 100 hours, more preferably 10 to 30 hours, especially about 20 hours. After cooling down, a second heat treatment is preferably carried out, in the range from 900 to 1300° C, preferably at about 1100° C, for a suitable time, preferably 1 to 30 hours, especially about 20 hours.

Alternatively, the element powders or preliminary alloy powders can be melted together in an induction oven. It is then possible in turn to perform heat treatments as specified above.

Processing via melt spinning is also possible. This allows obtaining a more homogeneous element distribution which leads to an improved magnetocaloric effect; cf. Rare Metals, Vol. 25, October 2006, pages 544 to 549. In the process described there, the starting elements are first induction-melted in an argon gas atmosphere and then sprayed in the molten state through a nozzle onto a rotating copper roller. This is followed by sintering at 1000° C and slow cooling to room temperature. In addition, reference may be made to US 8,211,326 and US 2011/0037342 for the production.

Preference is given to a process for producing the inventive magnetocaloric materials comprises the following steps
(a) reacting the starting materials in a stoichiometry which corresponds to the magnetocaloric material in the solid and/or liquid phase obtaining a solid or liquid reaction product,
(b) if the reaction product obtained in step (a) is in the liquid phase, transferring the liquid reaction product from step (a) into the solid phase obtaining a solid reaction product,
(c) optionally shaping of the reaction product from step (a) or (b)
(d) sintering and/or heat treating the solid product from step (a), (b) or (c), and
(e) quenching the sintered and/or heat treated product of step (d) at a cooling rate of at least 10 K/s., and
(f) optionally shaping of the product of step (e).
According to one preferred embodiment of the present invention step (c) shaping of the reaction product from step (a) or (b) is performed.

In step (a) of the process, the elements and/or alloys which are present in the magnetocaloric material are converted in the solid or liquid phase in a stoichiometry which corresponds to the material. Preference is given to performing the reaction in step a) by combined heating of the elements and/or alloys in a closed vessel or in an extruder, or by solid phase reaction in a ball mill. Particular preference is given to performing a solid phase reaction, which is effected especially in a ball mill. Such a reaction is known in principle; c.f. the documents previously cited. Typically, powders of the individual elements or powders of alloys of two or more of the individual elements which are present in the magnetocaloric material are mixed in pulverized or granular form in suitable proportions by weight. If necessary, the mixture can additionally be ground in order to obtain a microcrystalline powder mixture. This powder mixture is preferably mechanically impacted in a ball mill, which leads to further cold welding and also good mixing, and to a solid phase reaction in the powder mixture.

Alternatively, the elements are mixed as a powder in the selected stoichiometry and then melted. The combined heating in a closed vessel allows the fixing of volatile elements and control of the stoichiometry. Specifically in the case of use of phosphorus, this would evaporate easily in an open system.

Step (a) is preferably performed under inert gas atmosphere.

If the reaction product obtained in step (a) is in the liquid phase, the liquid reaction product from step (a) is transferred into the solid phase obtaining a solid reaction product in step (b).

The reaction is followed by sintering and/or heat treatment of the solid in step (d), for which one or more intermediate steps can be provided. For example, the solid obtained in step (a) can be subjected to shaping in step (c) before it is sintered and/or heat treated.

For example, is possible to send the solid obtained from the ball mill to a melt-spinning process. Melt-spinning processes are known per se and are described, for example, in Rare Metals, Vol. 25, October 2006, pages 544 to 549, and also in US 8,211,326 and WO 2009/133049. In these processes, the composition obtained in step (a) is melted and sprayed onto a rotating cold metal roller. This spraying can be achieved by means of elevated pressure upstream of the spray nozzle or reduced pressure downstream of the spray nozzle. Typically, a rotating copper drum or roller is used, which can additionally optionally be cooled. The copper drum preferably rotates at a surface speed of 10 to 40 m/s, especially from 20 to 30 m/s. On the copper drum, the liquid composition is cooled at a rate of preferably from 10² to 10⁷ K/s, more preferably at a rate of at least 10⁴ K/s, especially with a rate of from 0.5 to 2*10⁶ K/s.

The melt-spinning, like the reaction in step (a), can be performed under reduced pressure or under an inert gas atmosphere.
The melt-spinning achieves a high processing rate, since the subsequent sintering and heat treatment can be shortened. Specifically on the industrial scale, the production of the magnetocaloric materials thus becomes significantly more economically viable. Spray drying also leads to a high processing rate. Particular preference is given to performing melt spinning.

Melt spinning can be performed to transfer the liquid reaction product obtained from step (a) into a solid according to step (b), but it is also possible that the melt spinning is performed as shaping step (c). According to one embodiment of the present invention one of steps (a) and (b) comprises melt spinning.

Alternatively, in step (b), spray cooling can be carried out, in which a melt of the composition from step (a) is sprayed into a spray tower. The spray tower may, for example, additionally be cooled. In spray towers, cooling rates in the range from 10³ to 10⁵ K/s, especially about 10⁴ K/s, are frequently achieved.

In step (c) optionally shaping of the reaction product of step (a) or (b) is performed. Shaping of the reaction products may be performed by the shaping methods known to the person skilled in the art like pressing, molding, extrusion etc.

Pressing can be carried out, for example, as cold pressing or as hot pressing. The pressing may be followed by the sintering process described below.

In the sintering process or sintered metal process, the powders of the magnetocaloric material are first converted to the desired shape of the shaped body, and then bonded to one another by sintering, which affords the desired shaped body. The sintering can likewise be carried out as described below.

It is also possible in accordance with the invention to introduce the powder of the magnetocaloric material into a polymeric binder, to subject the resulting thermoplastic molding material to a shaping, to remove the binder and to sinter the resulting green body. It is also possible to coat the powder of the magnetocaloric material with a polymeric binder and to subject it to shaping by pressing, if appropriate with heat treatment.

According to the invention, it is possible to use any suitable organic binders which can be used as binders for magnetocaloric materials. These are especially oligomeric or polymeric systems, but it is also possible to use low molecular weight organic compounds, for example sugars.

The magnetocaloric powder is mixed with one of the suitable organic binders and filled into a mold. This can be done, for example, by casting or injection molding or by extrusion. The polymer is then removed catalytically or thermally and sintered to such an extent that a porous body with monolith structure is formed.

Hot extrusion or metal injection molding (MIM) of the magnetocaloric material is also possible, as is construction from thin sheets which are obtainable by rolling processes. In the case of injection molding, the channels in the monolith have a conical shape, in order to be able to remove the moldings from the mold. In the case of construction from sheets, all channel walls can run in parallel.

Steps (a) to (c) are followed by sintering and/or heat treatments of the solid, for which one or more intermediate steps can be provided.

The sintering and/or heat treatments of the solid is effected in step (d) as described above. In the case of use of the melt-spinning process, the period for sintering or heat treatments can be shortened significantly, for example toward periods of from 5 minutes to 5 hours, preferably from 10 minutes to 1 hour. Compared to the otherwise customary values of 10 hours for sintering and 50 hours for heat treatment, this results in a major time advantage. The sintering/heat treatment results in partial melting of the particle boundaries, such that the material is compacted further.

The melting and rapid cooling comprised in steps (a) to (c) thus allows the duration of step (d) to be reduced considerably. This also allows continuous production of the magnetocaloric materials.

The sintering and/or heat treatment of the compositions obtained from one of steps (a) to (c) is effected in step (d). The maximal temperature of the sintering (T < melting point) is a strong function of composition. Extra Mn decreases the melting point and extra Si increases it. Preferably the compositions are first sintered at a temperature in the range from 800 to 1400°C, more prefered in the range from 900 to 1300°C. For shaped bodies/solids, the sintering is more preferably effected at a temperature in the range from 1000 to 1300 °C, especially from 1000 to 1200°C. The sintering is performed preferably for a period of from 1 to 50 hours, more preferably from 2 to 20 hours, especially from 5 to 15 hours (step d1). After sintering the compositions are preferably heat treated at a temperature in the range of from 500 to 1000 °C, preferably in the range of from 700 to 1000 °C, but even more preferred are the aforementioned temperature ranges outside the range of 800 to 900 °C, i.e the heat treatment is preferably performed at a temperature T wherein 700 °C < T < 800 °C and 900 °C < T < 1000 °C. The heat treatment is performed preferably for a period in the range from 1 to 100 hours, more preferably from 1 to 30 hours, especially from 10 to 20 hours (step d2). This heat treatment may then followed by a cool down to room temperature, which is preferably carried out slowly (step d3). An additional second heat treatment may be carried out at temperatures in the range of from 900 to 1300 °C, preferably in the range of from 1000 to 1200°C for a suitable period like, preferably 1 to 30 hours, preferably 10 to 20 hours (step d4).

The exact periods can be adjusted to the practical requirements according to the materials. In the case of use of the melt-spinning process, the period for sintering or heat treatment can be shortened significantly, for example to periods of from 5 minutes to 5 hours, preferably from 10 minutes to 1 hour. Compared to the otherwise customary values of 10 hours for sintering and 50 hours for heat treatment, this results in a major time advantage.

The sintering/heat treatment results in partial melting of the particle boundaries, such that the material is compacted further.

The melting and rapid cooling in step (b) or (c) thus allows the duration of step (d) to be reduced considerably. This also allows continuous production of the magnetocaloric materials.

Preferably step (d) comprises the steps
(d1) sintering,
(d2) first heat treatment,
(d3) cooling, and
(d4) second heat treatment.

Steps (d1) to (d4) may be performed as described above.

In step (e) quenching the sintered and/or heat treated product of step (d) at a cooling rate of at least 10 K/s, preferably of at least 100 K/s is performed. The thermal hysteresis and the transition width can be reduced significantly when the magnetocaloric materials are not cooled slowly to ambient temperature after the sintering and/or heat treatments, but rather are quenched at a high cooling rate. This cooling rate is at least 10 K/s, preferably at least 100 K/s.

The quenching can be achieved by any suitable cooling processes, for example by quenching the solid with water or aqueous liquids, for example cooled water or ice/water mixtures. The solids can, for example, be allowed to fall into ice-cooled water. It is also possible to quench the solids with subcooled gases such as liquid nitrogen. Further processes for quenching are known to those skilled in the art. The controlled and rapid character of the cooling is advantageous especially in the temperature range between 800 and 900°C, i.e. it is preferred to keep the exposure of the material to temperatures in the range between 800 and 900°C as short as possible.

The rest of the production of the magnetocaloric materials is less critical, provided that the last step comprises the quenching of the sintered and/or heat treated solid at the large cooling rate.

In step (f) the product of step (e) may be shaped. The product of step (e) may be shaped by any suitable method known by the person skilled in the art, e.g. by bonding with epoxy resin or any other binder. Performing shaping step (f) is especially preferred if the product of step (e) is obtained in form of a powder or small particles.

The inventive magnetocaloric materials can be used in any suitable applications. For example, they can be used in cooling systems like refrigerators and climate control units, heat exchangers, heat pumps or thermoelectric generators. Particular preference is given to use in cooling systems. Further object of the present invention are cooling systems, heat exchangers, heat pumps and thermoelectric generators comprising at least one inventive magnetocaloric material as described above. The invention is hereafter illustrated in detail by examples and by referring to state of the art in the magnetic refrigeration field.

### Examples

### A) Preparation of the magnetocaloric materials

All the examples described hereafter are synthesized according to the same protocol. Stoichiometric quantities of Mn flakes, B flakes, and powders of Fe₂P, P, and Si were ground in a planetary ball mill for 10 h with a ball to sample weight ratio of 4. The resulting powders were then pressed into pellets and sealed in quartz ampules under Ar atmosphere of 200 mbar. The heat treatment was performed via a multiple steps process: first, a sintering at 1100 °C for 2 hours, followed by a first 20 hours heat treatment at 850 °C was performed. Subsequently the samples were cooled down to room temperature in the furnace. Finally, the samples were heat treated at 1100 °C for 20 hours followed by rapid quenching of the samples by dropping the hot quartz ampules into water at room temperature.

The compositions of the materials prepared are summarized in Table 1.

**Table 1: Compositions**

| Example | Formula | z |
|---|---|---|
| 1 (comparative) | MnFe_{0.95}P_{2/3-z}B_{z}Si_{1/3} | 0.00 |
| 2 (comparative) | Mn_{1.1}Fe_{0.85}P_{2/3-z}B_{z}Si_{1/3} | 0.00 |
| 3 (inventive) | Mn_{1.1}Fe_{0.85}P_{2/3-z}B_{z}Si_{1/3} | 0.07 |
| 4 (comparative) | Mn_{1.15}Fe_{0.8}P_{2/3-z}B_{z}Si_{1/3} | 0.04 |
| 5 (comparative) | Mn_{1.15}Fe_{0.8}P_{2/3-z}B_{z}Si_{1/3} | 0.05 |
| 6 (inventive) | Mn_{1.15}Fe_{0.8}P_{2/3-z}B_{z}Si_{1/3} | 0.06 |
| 7 (inventive) | Mn_{1.15}Fe_{0.8}P_{2/3-z}B_{z}Si_{1/3} | 0.07 |
| 8 (comparative) | Mn_{1.3}Fe_{0.65}P_{2/3-z}B_{z}Si_{1/3} | 0.00 |
| 9 (comparative) | Mn_{1.3}Fe_{0.65}P_{2/3-z}B_{z}Si_{1/3} | 0.02 |
| 10 (comparative) | Mn_{1.3}Fe_{0.65}P_{2/3-z}B_{z}Si_{1/3} | 0.04 |
| 11 (inventive) | Mn_{1.3}Fe_{0.65}P_{2/3-z}B_{z}Si_{1/3} | 0.06 |
| 12 (comparative) | Mn_{1.3}Fe_{0.65}P_{0.5}Si_{0.5} | |
| 13 (comparative) | Mn_{1.25}Fe_{0.7}P_{0.5}Si_{0.5} | |

If B is not present, the composition can be given very accurately. However, especially for very small quantities of B, it is difficult to determine the value of z very precisely. This has to do with the affinity of B to oxygen. If oxygen is present in the sample, which is almost inevitable, part of the B will react to B₂O₃ which is volatile and thus will not enter the compound. Usually the error of z is about ± 0.01.

### B) Measurements

The specific heat of the examples was measured in a differential scanning calorimeter in zero field at a sweep rate of 10 Kmin⁻¹. For all the magnetocaloric materials listed in table 1, the magnetic transition is accompanied by a symmetrical specific heat peak indicating that we are dealing with first order transitions, that is to say with Giant-magnetocaloric materials as described in K. A. Geschneidner Jr., V.K. Pecharsky and A. O. Tsokol, Rep. Prog. Phys. 68, 1479 (2005).

The magnetic properties of the examples were determined in a Quantum Design MPMS 5XL SQUID magnetometer.

The entropy change was derived on the basis of isofield magnetization measurements and the use of the so-called Maxwell relation (see A. M. G. Carvalho et al., J. Alloys Compd. 509, 3452 (2011)).

ΔT_{ad} was measured by a direct method on a home-made device. Magnetic field changes of 1.1 T were applied by moving/removing (1.1 Ts⁻¹) the samples from a magnetic field generated by a permanent magnet. A relaxation time of 4 s was used between each field changes, and thus, the duration of a full magnetization/demagnetization cycle was 10 s. The starting temperature of each cycle was externally controlled and swept between 250 K and 320 K at a rate of 0.5 Kmin⁻¹. It should be noted that the time required for the ΔT_{ad} to take place is generally of the order of 1 s or less, almost instantaneous compared to the sweeping rate.

The structural parameters were studied by collecting x-ray diffraction patterns at various temperatures in zero magnetic field in a PANalytical X-pert Pro diffractometer equipped with an Anton Paar TTK450 low temperature chamber. Structure determination and refinements were performed with the FullProf software (see http://www.ill.eu/sites/fullprof/index.html) and show that all the samples listed in table 1 crystallize in the hexagonal Fe₂P-type structure (space group *P*_{6̅2*m*})_{.}

### C) Results

Fig. 1A) to C) show the magnetization data measured in a field of B = 1 T upon cooling (open symbols) and upon heating (closed symbols) at a sweep rate of 1 Kmin⁻¹. These data illustrate the capability of boron substitution to reduce the hysteresis while keeping the saturation magnetization unmodified. These results are discussed in respect with the parameters proposed in US 2011/0167837, US 2011/0220838 and CN 102881393 A. The following observations can be made:

Fig. 1A): The thermal hysteresis of MnFe_{0.95}P_{2/3}Si_{1/3} (example 1; squares) is about 77 K. An increase of the manganese content to Mn_{1.1}Fe_{0.85}P_{2/3}Si_{1/3} (example 2; circles) leads to a hysteresis of about 62 K, that is to say a decrease of the hysteresis by about -2 K per percent of manganese. But in the same time the magnetization values in the ferromagnetic state are decreased, which is an undesirable secondary consequence of Mn addition. In contrast, the substitution by boron in Mn_{1.1}Fe_{0.85}P_{2/3}Si_{1/3} leads to a very small hysteresis without any further decrease of the saturation magnetization, as shown by Mn_{1.1}Fe_{0.85}P_{0.60}B_{0.07}Si_{1/3} (example 3, triangles) having a hysteresis of 1 K. The average hysteresis decrease is thus about -10 K per percent of boron.

Fig. 1B): In order to have Curie temperatures below room temperature, starting from MnFe_{0.95}P_{2/3}Si_{1/3} (example 1 shown in Fig. 1A), the Manganese content has to be increased, while the Silicon content must be kept at about 1/3. The Mn_{1.15}Fe_{0.8}P_{2/3-z}B_{z}Si_{1/3} series (z = 0.04, example 4, squares; z = 0.05, example 5, circles ; z = 0.06, example 6, triangles ; and z = 0.07, example 7, diamonds) is a good example of this possibility. The compositions having the desired properties (limited hysteresis, sharpness of the transition) correspond to z = 0.06 and z = 0.07.

Fig. 1C): In the Mn_{1.3}Fe_{0.65}P_{2/3-z}B_{z}Si_{1/3} series (z = 0.00, example 8, squares; z = 0.02, example 9, circles ; z = 0.04, example 10, triangles ; and z = 0.06 example 11 diamonds) a similar result is obtained. The substitution of small fractions of P by B leads to better properties, in particular to reduced hysteresis, but to obtain materials showing the desired small hysteresis it is necessary that a minimum content of B is present; the composition having a limited hysteresis corresponds to z = 0.06 .

It appears that boron substitution is more efficient than the parameters proposed in US 2011/0167837 to control the hysteresis. In particular, in all the examples displayed in the Fig. 1A) to 1C), the substitution of phosphorous by boron does not affect the magnetization values in the ferromagnetic state, while it significantly reduces the thermal hysteresis.

Fig. 2A) shows a set of M_{B}(T) curves for Mn_{1.15}Fe_{0.8}P_{2/3-0.07}B_{0.07}Si_{1/3} (example 7) starting with B= 0.05 T and then at different fields between 0.25 T and 2 T (increments of 0.25 T), measured upon warming with a sweeping rate of 1 Kmin⁻¹. A large magnetization jump of about 74 Am²kg⁻¹ is found at the magnetic phase transition in B = 1 T leading to a large magnetocaloric effect in this temperature range. The sensitivity of the magnetic phase transition in respect to the magnetic field, the dTc/dB of example 7 is shown in Fig. 2B. The squares correspond to the experimental T_{C}s, the line is a linear fit. dT_{C}/dB of example 7 amounts to +4.9 +/- 0.2 KT⁻¹ which is higher than for (MnₓFe₁₋ₓ)₂₊ᵤP_{1-y}Si_{y} compounds. In particular this value is significantly higher (+50 %) than the +3.25 ± 0.25 KT⁻¹ reported for the Boron-free material Mn_{1.25}Fe_{0.7}P_{0.5}Si_{0.5} [N. H. Dung et al., Phys. Rev. B 86, 045134 (2012)]. This improvement of the dT_{C}/dB is in agreement with the objective of the invention and will result in large adiabatic temperature changes in these boron substituted compounds.

Fig. 3 presents a panel of ΔS curves for some inventive materials (examples 3, 6, 7 and 11) for field changes of 1 T (open symbols) and 2 T (closed symbols). The maximal values of |ΔS| for ΔB = 1 T are in the range 8-10 J kg⁻¹K⁻¹, that is to say about 3-4 times higher than the elemental gadolinium, this fact confirms that these materials display a so-called "giant" magnetocaloric effect (see review K. A. Geschneidner Jr., V.K. Pecharsky and A. O. Tsokol, Rep. Prog. Phys. 68, 1479 (2005)). It should be noted that for boron substituted samples the |ΔS| values in ΔB= 1 T are similar or even higher than the compositions shown in US2011/0220838A and US 2011/0167837. Accordingly, the improvements of dT_{C}/dB, ΔT_{ad} and the mechanical stability in Boron substituted samples are obtained without any reduction of the ΔS performances. Finally, let us notice that the ΔS presented here are based on M_{B}(T) measurements which is a technique known by the people skilled in the art to not face to the spike problem (i.e. anomalous huge ΔS values obtained during the derivation of ΔS on the basis of M_{T}(B) curves). Thus, our ΔS cannot be compared to the ΔS values presented in CN 102881393 where phase coexistence features can clearly be observed (obvious double step behavior on M_{T}(B) curves on the Fig. 5a), 6a) and 6b) of CN 102881393).

Fig. 4A) shows the adiabatic temperature changes ΔT_{ad} of the examples 3 and 12. Maximal values of about 2.5 K are obtained in the present inventive material, example 3, which is very close to the highest values reported so-far in giant magnetocaloric materials around room temperature (see review K. A. Geschneidner Jr., V.K. Pecharsky and A. O. Tsokol, Rep. Prog. Phys. 68, 1479 (2005)). These ΔT_{ad} values are significantly higher than in a Boron free material based on a preferred composition of US 2011/0167837 (+45% improvement compared to example 12). It is worth noting that these measured ΔT_{ad} correspond to a fully reversible effect since they are determined during continuous cycling operations, see Fig. 4B) for example 3 (the squares correspond to the sample temperatures, the arrows mark the magnetic field changes). This is in strong contrast to "Giant" ΔT_{ad} values published recently, where the ΔT_{ad} measured during cycling operation is only one third of the non-reversible ΔT_{ad} value (see "Giant magnetocaloric effect driven by structural transitions", by J. Liu, T. Gottschall, et al. in Nature Mat. 11, 620 (2012)). For similar reasons (too large hysteresis), the compositions displayed in CN 102881393A , which show a large thermal hysteresis from 12 K to 27 K, will not have any significant reversible ΔT_{ad} in intermediate magnetic field (for ΔB ≤ 2T) ; that is to say these compositions cannot be used in a cyclic application like a magnetic refrigerator.

Fig. 5A) displays the ratio between the c and a cell parameters determined by x-ray diffraction for two inventive materials with Si= 1/3, examples 6, 7 and one comparative material example 13 from the preferred composition of US 2011/0167837. The unit cell of the preferred compositions of formula (MnₓFe₁₋ₓ)₂₊ᵤP_{1-y-z}Si_{y}B_{z} is hexagonal, the "structural" changes at the magnetic phase transition are not isotropic. For examples 6 (squares) and 7 (circles), a jump of the cell parameters at T_{C} is observed and appears to be almost as pronounced as in a composition without boron (Mn_{1.25}Fe_{0.7}P_{0.5}Si_{0.5}; example 13, triangles). But as shown in Fig. 5B) for the boron substituted samples (examples 6 and 7, squares and circles) no jump of the cell volume was observed, while there was a sizable ΔV/V of about +0.25 % in Mn_{1.25}Fe_{0.7}P_{0.5}Si_{0.5} (triangles). The ΔV of about 0 observed for boron substituted samples turns out to be smaller than ΔV of (Mn,Fe)₂(P, As) based materials where ΔV/V= -0.44 % (see Jap. J. of Appl. Phy. 44, 549 (2005)), (Mn,Fe)₂(P, Ge) based materials where ΔV/V= +0.1 % (see J. Phys. Soc. Jpn. 75, 113707 (2006)) and (Mn,Fe)₂(P, Si) based materials where ΔV/V= +0.25 % (as aforesaid). To our knowledge, this is the first time that a ΔV of about 0 which is practically the mere thermal expansion, i.e. without any discontinuity like a jump or step in the temperature dependence, is observed at the first order transition of a giant MCE material.

This very small ΔV at T_{C} in boron substituted samples gives a good mechanical stability to these samples. The good mechanical stability has been confirmed by cycling the samples across the transition during direct ΔT_{ad} measurements. The shape of the sample for ΔT_{ad} measurements corresponds to a thin cylinder of 10 mm diameter and 1 mm thickness. Even after the 8000 cycles of magnetization/demagnetization used for the ΔT_{ad} measurement, the geometry of the boron substituted compositions remains intact and the mechanical integrity is maintained. It should be noted that the same experimental method has already been used to check the mechanical stability of giant MCE materials, for instance in La(Fe,Si)₁₃ based materials (Adv. Mat. 22, 3735 (2010)).

## Claims

1. A magnetocaloric material of the general formula (I)
(MnₓFe₁₋ₓ)₂₊ᵤ P_{1-y-z}Si_{y}B_{z}
wherein
0.55 ≤ x ≤ 0.75,
0.25 ≤ y < 0.4,
0.05 < z ≤ 0.2,
-0.1 ≤ u ≤ 0.05.

2. The magnetocaloric material according to claim 1, wherein 0.6 ≤ x ≤ 0.7.

3. The magnetocaloric material according to claim 1, wherein 0.3 ≤ y < 0.4.

4. The magnetocaloric material according to claims 1 to 3, wherein 0.052 ≤ z ≤ 0.1.

5. The magnetocaloric material according to any of claims 1 to 4, wherein -0.1 ≤ u ≤ 0.

6. The magnetocaloric material according to any of claims 1 to 5, wherein -0.06 ≤ u ≤ -0.04.

7. The magnetocaloric material according to any of claims 1 to 6, wherein 0.6 ≤ x ≤ 0.7, 0.3 ≤ y < 0.4 and 0.052 ≤ z ≤ 0.1.

8. The magnetocaloric material according to any of claims 1 to 7, which has a hexagonal crystalline structure of the Fe₂P type.

9. The magnetocaloric material according to any of claims 1 to 8, which shows a value of |ΔV/V| < 0.05 % at the magnetic phase transition determined by X-ray diffraction.

10. A process for producing the magnetocaloric materials according to any of claims 1 to 9 comprising the following steps:
(a) reacting the starting materials in a stoichiometry which corresponds to the magnetocaloric material in the solid and/or liquid phase obtaining a solid or liquid reaction product,
(b) if the reaction product obtained in step (a) is in the liquid phase, transferring the liquid reaction product from step (a) into the solid phase obtaining a solid reaction product,
(c) optionally shaping of the reaction product from step (a) or (b)
(d) sintering and/or heat treating the solid product from step (a), (b) or (c)
(e) quenching the sintered and/or heat treated product of step (d) at a cooling rate of at least 10 K/s , and
(f) optionally shaping of the product of step (e)

11. The process according to claim 10, wherein step (c) is performed.

12. The process according to claim 10 or 11, wherein the starting materials are selected from the elements Mn, Fe, P, B and Si and the alloys and compounds formed by said elements among each other.

13. The use of the magnetocaloric materials according to any of claims 1 to 9 in cooling systems, heat exchangers, heat pumps or thermoelectric generators.

14. Cooling systems, heat exchangers, heat pumps and thermoelectric generators comprising at least one magnetocaloric material according to any of claims 1 to 9.

## Patentansprüche

1. Magnetokalorisches Material der allgemeinen Formel (I)
(MnₓFe₁₋ₓ)₂₊ᵤP_{1-y-z}Si_{y}B_{z},
wobei
0,55 ≤ x ≤ 0,75,
0,25 ≤ y < 0,4,
0,05 < z ≤ 0,2,
-0,1 ≤ u ≤ 0,05.

2. Magnetokalorisches Material nach Anspruch 1, wobei 0,6 ≤ x ≤ 0,7.

3. Magnetokalorisches Material nach Anspruch 1, wobei 0,3 ≤ y < 0, 4 .

4. Magnetokalorisches Material nach Ansprüchen 1 bis 3, wobei
0,052 ≤ z ≤ 0,1.

5. Magnetokalorisches Material nach einem der Ansprüche 1 bis 4, wobei -0,1 ≤ u ≤ 0.

6. Magnetokalorisches Material nach einem der Ansprüche 1 bis 5, wobei -0,06 ≤ u ≤ -0,04.

7. Magnetokalorisches Material nach einem der Ansprüche 1 bis 6, wobei 0,6 ≤ x ≤ 0,7, 0,3 ≤ y < 0,4 und 0,052 ≤ z ≤ 0,1.

8. Magnetokalorisches Material nach einem der Ansprüche 1 bis 7, das eine hexagonale kristalline Struktur des Fe₂P-Typs aufweist.

9. Magnetokalorisches Material nach einem der Ansprüche 1 bis 8, das einen durch Röntgenbeugung bestimmten Wert von |ΔV/V| < 0,05 % am magnetischen Phasenübergang zeigt.

10. Verfahren zur Herstellung der magnetokalorischen Materialien nach einem der Ansprüche 1 bis 9, das folgende Schritte umfasst:
(a) Umsetzen der Ausgangsstoffe in einer Stöchiometrie, die dem magnetokalorischen Material entspricht, in der Fest- und/oder Flüssigphase zum Erhalt eines festen oder flüssigen Reaktionsprodukts,
(b) dann, wenn das in Schritt (a) erhaltene Umsetzungsprodukt in der Flüssigphase vorliegt, Überführen des flüssigen Umsetzungsprodukts aus Schritt (a) in die feste Phase zum Erhalt eines festen Umsetzungsprodukts,
(c) gegebenenfalls Formen des Umsetzungsprodukts aus Schritt (a) oder (b),
(d) Sintern und/oder Tempern des festen Produkts aus Schritt (a), (b) oder (c),
(e) Abschrecken des gesinterten und/oder getemperten Produkts aus Schritt (d) mit einer Abkühlgeschwindigkeit von mindestens 10 K/s und
(f) gegebenenfalls Formen des Produkts aus Schritt (e).

11. Verfahren nach Anspruch 10, bei dem Schritt (c) durchgeführt wird.

12. Verfahren nach Anspruch 10 oder 11, bei dem die Ausgangsstoffe aus den Elementen Mn, Fe, P, B und Si und den durch die Elemente untereinander gebildeten Legierungen und Verbindungen ausgewählt werden.

13. Verwendung der magnetokalorischen Materialien nach einem der Ansprüche 1 bis 9 in Kühlsystemen, Wärmetauschern, Wärmepumpen oder thermoelektrischen Generatoren.

14. Kühlsysteme, Wärmetauscher, Wärmepumpen oder thermoelektrische Generatoren, enthaltend mindestens ein magnetokalorisches Material nach einem der Ansprüche 1 bis 9.

## Revendications

1. Matériau magnétocalorique de formule générale (I)
(MnₓFe₁₋ₓ)₂₊ᵤP_{1-y-z}Si_{y}B_{z}
dans laquelle
0,55 ≤ x ≤ 0,75,
0,25 ≤ y < 0,4,
0,05 < z ≤ 0,2,
-0,1 ≤ u ≤ 0,05.

2. Matériau magnétocalorique selon la revendication 1, dans lequel 0,6 ≤ x ≤ 0,7.

3. Matériau magnétocalorique selon la revendication 1, dans lequel 0,3 ≤ y < 0,4.

4. Matériau magnétocalorique selon les revendications 1 à 3, dans lequel 0,052 ≤ z ≤ 0,1.

5. Matériau magnétocalorique selon l'une quelconque des revendications 1 à 4, dans lequel -0,1 ≤ u ≤ 0.

6. Matériau magnétocalorique selon l'une quelconque des revendications 1 à 5, dans lequel -0,06 ≤ u ≤ -0,04.

7. Matériau magnétocalorique selon l'une quelconque des revendications 1 à 6, dans lequel 0,6 ≤ x ≤ 0,7, 0,3 ≤ y < 0,4 et 0,052 ≤ z ≤ 0,1.

8. Matériau magnétocalorique, selon l'une quelconque des revendications 1 à 7, qui a une structure cristalline hexagonale du type Fe₂P.

9. Matériau magnétocalorique, selon l'une quelconque des revendications 1 à 8, qui présente une valeur de |ΔV/V| < 0,05 % au niveau de la transition de la phase magnétique, déterminée par une diffraction de rayons X.

10. Processus de production des matériaux magnétocaloriques, selon l'une quelconque des revendications 1 à 9, comprenant les étapes suivantes :
(a) faire réagir les matériaux de départ dans une stoechiométrie qui correspond au matériau magnétocalorique dans la phase solide et/ou liquide, en obtenant un produit réactionnel solide ou liquide,
(b) si le produit réactionnel obtenu à l'étape (a) est sous la forme liquide, transférer le produit réactionnel liquide issu de l'étape (a) dans la phase solide, en obtenant un produit réactionnel solide,
(c) en option, façonner le produit réactionnel issu des étapes (a) ou (b)
(d) fritter et/ou traiter par la chaleur le produit solide issu des étapes (a), (b) ou (c),
(e) effectuer l'extinction du produit fritté et/ou thermo-traité de l'étape (d) à une vitesse de refroidissement d'au moins 10 K/s, et
(f) en option, façonner le produit de l'étape (e).

11. Processus selon la revendication 10, dans lequel on exécute l'étape (c).

12. Processus selon les revendications 10 ou 11, dans lequel les matériaux de départ sont choisis parmi les éléments Mn, Fe, P, B et Si ainsi que les alliages et composés formés par lesdits éléments entre eux.

13. Utilisation des matériaux magnétocaloriques, selon l'une quelconque des revendications 1 à 9, dans des systèmes de refroidissement, échangeurs de chaleur, pompes à chaleur ou générateurs thermoélectriques.

14. Systèmes de refroidissement, échangeurs de chaleur, pompes à chaleur et générateurs thermoélectriques comprenant au moins un matériau magnétocalorique selon l'une quelconque des revendications 1 à 9.
